



US008486235B2

(12) **United States Patent**  
**Hillebrand**

(10) **Patent No.:** **US 8,486,235 B2**  
(45) **Date of Patent:** **\*Jul. 16, 2013**

(54) **ALKALINE ZINC-NICKEL BATH**(75) Inventor: **Ernst-Walter Hillebrand**, Wickede (DE)(73) Assignee: **EWH Industrieanlagen GmbH & Co. KG (DE)**

(\* ) Notice: Subject to any disclaimer, the term of this patent is extended or adjusted under 35 U.S.C. 154(b) by 23 days.

This patent is subject to a terminal disclaimer.

(21) Appl. No.: **12/896,673**(22) Filed: **Oct. 1, 2010**(65) **Prior Publication Data**

US 2011/0031127 A1 Feb. 10, 2011

**Related U.S. Application Data**

(60) Continuation of application No. 12/030,750, filed on Feb. 13, 2008, now Pat. No. 7,807,035, which is a continuation of application No. 10/618,352, filed on Jul. 11, 2003, now abandoned, which is a division of application No. 09/744,706, filed as application No. PCT/EP99/05443 on Jul. 29, 1999, now Pat. No. 6,602,394.

(30) **Foreign Application Priority Data**

Jul. 30, 1998 (DE) ..... 198 34 353

(51) **Int. Cl.**  
**C25B 9/10** (2006.01)(52) **U.S. Cl.**  
USPC ..... 204/252(58) **Field of Classification Search**

USPC ..... 205/246, 252; 204/252

See application file for complete search history.

(56) **References Cited**

## U.S. PATENT DOCUMENTS

|                |         |                          |
|----------------|---------|--------------------------|
| 3,660,170 A    | 5/1972  | Rampel                   |
| 3,718,549 A    | 2/1973  | Du Rose et al.           |
| 4,192,908 A    | 3/1980  | Himy et al.              |
| 4,469,564 A    | 9/1984  | Okinaka et al.           |
| 4,832,812 A    | 5/1989  | Brown                    |
| 4,889,602 A    | 12/1989 | Oshima et al.            |
| 5,162,079 A    | 11/1992 | Brown                    |
| 5,310,465 A    | 5/1994  | Vaughan                  |
| 5,403,460 A    | 4/1995  | Sala et al.              |
| 5,405,523 A    | 4/1995  | Eckles                   |
| 5,417,840 A    | 5/1995  | Block et al.             |
| 5,883,762 A    | 3/1999  | Calhoun et al.           |
| 6,602,394 B1 * | 8/2003  | Hillebrand ..... 205/246 |

## FOREIGN PATENT DOCUMENTS

|    |              |        |
|----|--------------|--------|
| DE | 925 264      | 3/1955 |
| DE | 33 10 730 A1 | 3/1984 |
| DE | 40 35 316 C2 | 5/1992 |
| DE | 37 12 511 C3 | 6/1995 |
| EP | 0410919 A1   | 1/1991 |

(Continued)

## OTHER PUBLICATIONS

Makoto Nonomura, Cyanide Formation in an Alkaline noncyanide Zinc Plating Bath, Jun. 1994.

(Continued)

Primary Examiner — Kishor Mayekar

(74) Attorney, Agent, or Firm — Cook Alex Ltd.

(57) **ABSTRACT**

The anode is separated from the alkaline electrode to avoid undesirable secondary reactions in an alkali zinc nickel electroplating bath.

**4 Claims, 1 Drawing Sheet**

## FOREIGN PATENT DOCUMENTS

|    |           |    |         |
|----|-----------|----|---------|
| EP | 0483937   | A1 | 10/1991 |
| GB | 1 349 735 |    | 4/1974  |
| GB | 1 602 404 |    | 11/1981 |
| JP | 58093886  | A  | 6/1983  |
| JP | 58093899  |    | 6/1983  |
| JP | 59193295  |    | 11/1984 |
| JP | 2175894   |    | 7/1990  |
| JP | 04-009493 |    | 1/1992  |
| JP | 4017693   |    | 1/1992  |
| JP | 04-052296 |    | 2/1992  |
| JP | 04-44374  |    | 4/1992  |
| JP | 4176893   |    | 6/1992  |
| JP | 04-259393 |    | 9/1992  |
| JP | 5009776   |    | 1/1993  |
| JP | 5009799   |    | 1/1993  |
| JP | 5128533   |    | 5/1993  |

|    |                |         |
|----|----------------|---------|
| JP | 10130878       | 5/1998  |
| JP | WO/98/40539    | 5/1998  |
| WO | PCT/EP99/05443 | 10/2000 |

## OTHER PUBLICATIONS

A.V. Ryabchenkov, Electrodeposition of zinc-nickel Alloys from electrolytes Containing Polyethylenepolyamine as a Complexing Agent, Nov. 16, 1972.  
A. Moebius, Maintenance of Electroplating and Pickling Baths—The Key for the Minimization of Waste, Jan. 1993.  
Wayne Roberts, Inert Anode for Chloride Zinc Plating, Jan. 1997.  
Von Andreas Zahl, Sulingen, Quo vadis Galvanotechnik, Mar. 4, 1998.

\* cited by examiner



**1**  
**ALKALINE ZINC-NICKEL BATH**

**BACKGROUND OF THE INVENTION**

The invention relates to an electroplating bath for plating zinc-nickel coatings, having an anode, a cathode and an alkaline electrolyte.

It is known to coat electrically conductive materials with zinc-nickel alloys in order to improve their resistance to corrosion. To do this, it is customary to use an acidic electrolyte bath, for example, with a sulfate, chloride, fluoropromate [sic] or sulfamate electrolyte. In these processes, it is very difficult and, in practice, generally impossible, in terms of control technology, to achieve a uniform thickness of the zinc-nickel coating on the material to be coated.

For this reason, the alkaline zinc-nickel electroplating baths which are disclosed in German Patent 37 12 511 have recently been used, having, for example, the following composition:

---

11.3 g/l ZnO  
4.1 g/l NiSO<sub>4</sub>·6H<sub>2</sub>O  
120 g/l NaOH  
5.1 g/l polyethyleneimine.

---

The amines contained in the electroplating bath serve as complex formers for the nickel ions, which are otherwise insoluble in the alkaline medium. The composition of the baths varies depending on the manufacturer.

The electroplating baths are usually operated with insoluble nickel anodes. The zinc concentration is kept constant by the addition of zinc and the nickel concentration is kept constant by the addition of a nickel solution, for example, a nickel sulfate solution. However, after they have been operating for a few hours, the color of these baths changes from what was originally blue-violet to brown. After a few days or weeks, this discoloration becomes more intense and it is possible to detect a separation of the bath into two phases, the upper phase being dark brown. This phase causes considerable disruption to the coating of the workpieces, such as, for example, nonuniform layer thickness or blistering. It is therefore imperative for the bath to be continuously cleaned, i.e., for this layer to be skimmed off continuously. However, this is time-consuming and expensive.

Furthermore, after a few weeks of operation it is possible to detect cyanide in the baths. Cyanide pollution requires regular cleaning of the bath and special wastewater treatment, which has a considerable effect on the operating costs of the bath. This applies all the more so if the wastewater has a very high concentration of organics and, with a COD value of approximately 15,000 to 20,000 mg/l, makes cyanide detoxification more difficult. It is then only possible to adhere to statutory wastewater parameters (nickel 0.5 ppm and zinc 2 ppm) by the extensive addition of chemicals.

The formation of the second phase is attributable to a reaction of the amines, which in alkaline solution are converted at the nickel anodes to form nitriles (including to form cyanide). Moreover, on account of the amines being broken down, fresh complex former has to be continuously added to the bath, which increases the costs of the process.

Anodes other than nickel anodes cannot be used, since they dissolve in the alkaline electrolyte, which also has adverse effects on the quality of the coating.

**2**  
**BRIEF SUMMARY OF THE INVENTION**

In view of this background, the invention is based on the problem of providing an alkaline zinc-nickel electroplating bath which provides high-quality zinc-nickel coatings at low cost.

To solve this problem, the invention proposes separating the anode from the alkaline electrolyte by an ion exchange membrane.

10 This separation prevents the amines from reacting at the nickel anode, with the result that there are no undesirable secondary reactions which cause waste disposal problems or lead to a second phase of reaction products being deposited on the bath and adversely affect the quality of the zinc-nickel coating. The invention obviates the need for this layer to be skimmed off at high cost and to renew the bath. Furthermore, there is a considerable improvement in the quality of the coating.

20 The use of a cation exchange membrane made from a perfluorinated polymer has proven particularly advantageous, since such membranes have a negligible electrical resistance but a high chemical and mechanical resistance.

Furthermore, the cyanide poisoning of the wastewater no longer takes place, thus considerably simplifying the entire wastewater treatment. Furthermore, there is no need to top up the complex former in the electrolyte, since it is no longer broken down and its concentration in the bath remains approximately constant. As a result, the cost of the process 30 becomes considerably less expensive.

35 In the solution according to the invention, the zinc-nickel bath functions as catholyte. The anolyte used may, for example, be sulfuric acid or phosphoric acid. In the electroplating cell according to the invention, customary anodes, such as, for example, platinum-coated titanium anodes, are suitable as anode material, since they are no longer exposed to the basic zinc-nickel bath.

40 The present invention is explained in more detail with reference to the exemplary embodiment illustrated in the drawing, in which:

**BRIEF DESCRIPTION OF THE DRAWING**

45 FIG. 1 shows the diagrammatic structure of an electroplating bath according to the invention.

**DETAILED DESCRIPTION OF THE INVENTION**

50 FIG. 1 shows an electroplating cell 1 which has an anode 2 and a cathode 3, which is the workpiece to be coated. The catholyte 4 surrounding the cathode is alkaline and consists of a zinc-nickel electroplating bath of known composition, in which amines are added as complex formers for the nickel ions. The anolyte 5 surrounding the anode 2 may, for example, consist of sulfuric acid or phosphoric acid. Anolyte 5 and catholyte 4 are separated from one another by a perfluorinated cation exchange membrane 6. This membrane 6 allows unimpeded flux of current through the bath but prevents the catholyte 4, in particular the amines contained therein, from coming into contact with the anode 2, thus preventing the reactions which were extensively described in the introduction to the description, including the adverse effects of these reactions.

65 The invention claimed is:

1. Alkaline electroplating cell (1) for plating zinc-nickel coatings, having an anode (2) a cathode (3) and an alkaline

electrolyte comprising amines, wherein the anode is separated from the alkaline electrolyte by an ion exchange membrane (6).

2. Electroplating cell (1) according to claim 1, wherein the ion exchange membrane(6) comprises a perfluorinated cation 5 ion exchange membrane.

3. Electroplating cell (1) according to claims 1 or 2, characterized by sulfuric acid, phosphoric acid, methanesulfonic acid, amidosulfonic acid and/or phosphonic acid as anolyte 10 (5).

4. Electroplating cell (1) according to one of claims 1 or 2, wherein the anode comprises a platinum-coated titanium anode.

\* \* \* \* \*